# EUROPEAN PATENT SPECIFICATION

(11) **EP 1 735 384 B1**
(45) Date of publication and mention of the grant of the patent: **21.07.2010**
(21) Application number: 05718324.6
(22) Date of filing: 01.04.2005
(51) Int. Cl.: C09B 7/00, D06P 1/38, D06P 3/02, D06P 3/66

(54) **PROCESS FOR DYEING AND DYE MIXTURES**
FÄRBEVERFAHREN SOWIE FARBTOFFMISCHUNGEN
PROCÉDÉ DE TEINTURE ET MÉLANGES DE COLORANTS

(30) Priority: 06.04.2004 EP 04008292
(43) Date of publication of application: 27.12.2006
(73) Proprietor: Clariant Finance (BVI) Limited, Road Town, Tortola (VG)
(72) Inventor: NUSSER, Rainer, 79395 Neuenburg (DE); GISLER, Markus, CH-4310 Rheinfelden (CH)
(74) Representative: Jacobi, Carola
(86) International application number: PCT/IB2005/000846
(87) International publication number: WO 2005/097911

(56) References cited:
- EP-A- 0 922 735
- EP-A- 0 962 500
- EP-A- 1 275 700
- WO-A-95/32249

## Description

The present invention relates to a process for the bichromatic and/or trichromatic dyeing or printing hydroxy-group-containing or nitrogen-containing organic substrates with dye mixtures and also to such dye mixtures and hydroxy-group-containing or nitrogen-containing organic substrates dyed or printed therewith.

Trichromatic describes the additive colour mixing of suitable yellow- or orange-, red- and blue-dyeing dyes with which any desired shade in the visible spectrum can be obtained by suitably selecting the amount ratios for the dyes. However, it is possible to achive some shades by mixing only two colorants selected from a suitable yellow- or orange-, red- and blue-dyeing dye which is here called bichromatic dyeing.

Trichromatic and bichromatic dyeing is well known from the literature for various dye classes, for example from EP 83299, DE 2623178, EP 226982 and EP808940.

Optimum trichromatic or bichromatic performance of any yellow (or orange), red and blue dye mixture is crucially dependent on the neutral affinity and migration characteristics. Dyes having identical or very similar characteristics with regard to neutral affinity and migration are highly compatible with regard to trichromatic or bichromatic performance.

It is an object of the present invention to provide a trichromatic or bichromatic dyeing process and associated trichromatic or bichromatic dye mixtures consisting of at least one red component, at least one yellow component or orange component or one blue component whereby trichromatic or bichromatic dyeing with good fastnesses is obtained.

This object is achieved by a trichromatic or bichromatic dyeing process which is characterized by using a dye mixture comprising a red-dyeing compound of the formula (I) and at least one yellow-dyeing compound or orange-dyeing compound or one blue-dyeing compound.

In a further embodiment this object is achieved by a trichromatic dyeing process which is characterized by using a dye mixture comprising a red-dyeing compound of the formula (I) and at least one yellow-dyeing compound or orange-dyeing compound and at least one blue-dyeing compound.

Various auxiliaries, such as surface-active compounds, solubilising agents, thickeners, gel-forming substances, antioxidants, penetration agents, sequestering agents, buffers, light protection agents, care agents may additionally be present in the composition according to the invention.

Such auxiliaries are in particular wetting agents, antifoams, levelling agents, thickeners and plasticizers.

For the preparation of inks for printing processes suitable organic solvents or mixtures thereof are used. E.g. alcohols, ethers, esters, nitriles, carbonacidamides, cyclic amides, urea, sulfones and sulfone oxides.

Furthermore additional auxiliaries such as e.g. compounds, which adjust the viscosity and/ or the surface tension, may be added to the ink composition.

Suitable yellow-dyeing compounds or orange-dyei ng compounds for the inventive trichromatic or bichromatic process have the following formula (II) wherein
- R₄ and R₅: signify independently from each other H or -SO₃H,
- A: signifies a group of formula (i) or (ia)
wherein
- X: is a halogen radical and
- Y: signifies -CH=CH₂ or -CH₂CH₂-Z, wherein Z is a radical which can be eliminated by alkali,
- R₆ and R₇: signify independently from each other H; unsubstituted C₁₋₄alkyl or substituted C₁₋₄alkyl,
- B: signifies
wherein R₈ signifies C₁₋₄alkyl; -NH₂ or -NHC₁₋₄alkyl,
and the asterisk marks the bond to the -N=N- group.

A suitable radical Z which can be eliminated by alkali or under alkaline conditions, respectively, is for example chlorine; bromine or -OSO₃H or -SSO₃H or the alkali metal salt thereof; and by preference -OSO₃H or the alkali metal salt thereof.

Further suitable yellow-dyeing compounds or orange-dyeing compounds for the inventive trichromatic or bichromatic process have the following formula (IV) wherein
- R₁₃: signifies H; methyl; methoxy, ethoxy; -NHCONH₂ or -NHCOCH₃,
- R₁₄: signifies H; methyl; methoxy or ethoxy,
- RG: signifies
wherein
- R₁₅: signifies H or chlorine,
- Y: signifies -CH=CH₂ or -CH₂CH₂-Z, wherein Z is a radical which can be eliminated by alkali, and may be bonded in the position 4 or 5 with respect to the azo group.

Suitable blue-dyeing compounds for the inventive trichromatic or bichromatic process have the following formula (V) or (VI) in which
- R₂₁: is H or -COOH,
- each of R₂₂ and R₂₄: is independently H; -COOH; -SO₃H; -NHCOCH₃; -NHCOCHY₂- CH₂Y₁; -NHCOCY₂=CH₂ or -NHCOCH₂Y₁.
- R₂₃: -COOH,
- Y₁: is chlorine; bromine; -OSO₃H or -SSO₃H and
- Y₂: is H; chlorine or bromine.

Further suitable blue-dyeing compounds for the inventive trichromatic or bichromatic process have the following formula (VI) in which
- Y: signifies -CH=CH₂ or -CH₂CH₂-Z, wherein Z is a radical which can be eliminated by alkali,
- R₂₅: signifies H or -SO₃H,
- R₂₆: signifies H or -SO₃H.

Further suitable blue-dyeing compounds for the inventive trichromatic or bichromatic process have the following formula (VII) wherein
- each Y: has independently from each other the same meanings as defined above
- R₂₇ and R₂₈: are independently from each other H; unsubstituted C₁₋₄alkyl or substituted C₁₋₄alkyl.

A preferred bichromatic dyeing process is characterized by using a dye mixture comprising a red-dyeing compound of the formula (I) and at least one yellow-dyeing compound or orange-dyeing compound of the formula (II), (III) and/or (IV)

A further preferred bichromatic dyeing process is characterized by using a dye mixture comprising a red-dyeing compound of the formula (I) and at least one blue-dyeing compound as per the formula (V), (VI), and/or (VII).

A preferred trichromatic dyeing process is characterized by using a dye mixture comprising a red-dyeing compound of the formula (I) and at least one yellow (or orange)-dyeing compound of the formula (II), (III) and/or (IV) and at least one blue-dyeing compound as per the formula (V), (VI), and/or (VII).

A more preferred trichromatic dyeing process is characterized by using a dye mixture comprising at least one yellow (or orange)-dyeing compound of formula (IIa), (IIb) and/or (IIc) wherein A is or and/or at least one yellow-dyeing compounds or orange-dyeing compounds of formula (IVa) or (IVb) wherein RG is and/or at least one blue-dyeing compound of formula (Va) or (Vb) and/or at least one blue-dyeing compounds of formula (VIa) or (VIb) and/or at least one blue-dyeing compound of formula (VIIa)

It is to be noted that all compounds may also be present in salt form. Useful salts include in particular alkali metal, alkaline earth metal or ammonium salts or the salts of an organic amine.

It is likewise to be noted that the alkyl groups can be linear or branched.

Suitable groups Z which may be eliminated by alkali in the group -SO₂-CH₂CH₂-Z are chlorine; bromine; -OSO₃H or -SSO₃H.

Preferred hydroxy-group-containing or nitrogen-containing organic substrates are leather and fibrous materials, which comprise natural or synthetic polyamides and, particularly, natural or regenerated cellulose such as, cotton, viscose and spun rayon. The most preferred substrates are textile materials comprising cotton.

The compound of the formula (I) is prepared according to EP962500.

The yellow-dyeing compounds or orange-dyeing compounds are known from the state of the art and can therefore be produced according to the process given in the prior art. E.g. WO96/02593 and F.Lehr, Dyes Pigm. (1990),14(4),257.

The blue-dyeing compounds are also known from the state of the art and can therefore be produced according to the process given in the prior art. E.g. EP 99721, EP84314, W00168775, EP 149170, EP497174 and DE4241918.

This invention further provides dye mixtures for the trichromatic dyeing or printing of hydroxy-group-containing or nitrogen-containing organic substrates as defined in claim 6.

The inventive process for trichromatic dyeing or printing can be applied to all customary and known dyeing and printing processes, for example the continuous process, the exhaust process, the foam dyeing process and the ink-jet process.

The composition of the individual dye components in the trichromatic dye mixture used in the process according to the invention depends on the desired hue. For instance, a brown hue preferably utilizes 30-65% by weight of the yellow (or orange) component according to the invention, 10-30% by weight of the red component according to the invention and 10-30% by weight of the blue component according to the invention.

The red component, as described above, can consist of a single component or of a mixture of different red individual components.

The same applies to the yellow (or orange) and blue components.

The total amount of dyes in the process according to the invention is between 0.01 and 15% by weight, preferably between 1 and 10% by weight.

The present invention further provides hydroxy-group-containing or nitrogen-containing organic substrates dyed or printed by a dye mixture according to the invention.

The process according to the invention provides dyeings and prints having a homogeneous hue build-up throughout the entire hue spectrum with on-tone exhaustion, with a high bath exhaustion even in the case of fibres with low saturation and with a high dye build-up on fine fibres, particularly on microfibres.

The resulting dyeings or prints are notable for very high wet fastnesses, specifically the fastnesses in washing, perspiration and water. These good wet and fabrication fastnesses, which are in no way inferior to the fastness level of dyeings and prints with metal complexes, are obtained without aftertreatment. With an additional aftertreatment, these fastnesses are even exceeded.

These excellent results are provided by metal-free elements which meet the current and future ecological requirements of national institutes and regulations.

The tables which follow show some examples of the individual components of the dye mixtures which are used in the inventive trichromatic dyeing process.

**TABLE 1/ Examples 1-4**

| Examples of yellow-dyeing compounds or orange-dyeing compounds of formula (II') according to formula (II) | | | | |
|---|---|---|---|---|
| | | | | |

| **Ex.** | **R₄** | **R₅** | **A** | **Position -N=N-** |
|---|---|---|---|---|
| 1 | SO₃H | (3)-SO₃H | | 2 |
| 2 | SO₃H | (3)-SO₃H | | 2 |
| 3 | H | (4)-SO₃H | | 3 |
| 4 | SO₃H | (3)-SO₃H | | 2 |

**TABLE 2/ Examples 5-7**

| Examples of yellow-dyeing compounds or orange-dyeing compounds of formula according to formula (IV) | | | |
|---|---|---|---|
| | | | |

| **Ex.** | **Position** **-SO₂CH₂CH₂OSO₃H** | **G** | **RG'** |
|---|---|---|---|
| 5 | 4 | -NH₂ | |
| 6 | 3 | -CH₃ | |
| 7 | 4 | -CH₃ | |

The application examples hereinbelow serve to illustrate the present invention. Parts are by weight and % are weight-%, unless otherwise indicated. Temperatures are in degrees Celsius, unless otherwise indicated.

### APPLICATION EXAMPLE 1

A 20 g sample of bleached cotton knitting. is transferred in a solution of 16 g sodium sulfate in 200 ml water at 60°C,
0.5 % (calculated on the fabric weight) of a red dye of formula (I)
0.8 % of a yellow dye as per Example 4
0.5 % of a blue dye as per Formula Va and
portions of 0.3, 0.7 and 1 g of sodium carbonate are added at 60°C after 30, 45 respectively 60 minutes. The temperature is maintained during another 60 minutes. The dyed fabric is rinsed in hot distilled water during 2 minutes and in hot tap water during 1 minute. After being kept in 1000 ml distilled water at the boil for 20 minutes. the fabric is dried. It provides a brown cotton dyeing having good fastnesses.

### EXAMPLES 2-16

These examples are made analogous to Use Example 1, but by using dyestuff mixtures as mentioned below. The resulted shade is given in brackets.

### APPLICATION EXAMPLE 2 (olive shade)

0.2 % of a red dye of formula (I)
0.4 % of a yellow dye as per Example 4
0.6 % of a blue dye as per Formula Va

### APPLICATION EXAMPLE 3 (brown shade)

0.3 % of a red dye of formula (I)
0.9 % of a orange dye as per Example 6
0.6 % of a blue dye as per Formula V a

### APPLICATION EXAMPLE 4 (olive shade)

0.1 % of a red dye of formula (I)
0.5 % of a yellow dye as per Example 6
0.6 % of a blue dye as per Formula Va

### APPLICATION EXAMPLE 5 (brown shade)

0.5 % of a red dye of formula (I)
0.9 % of a yellow dye as per Example 4
0.3 % of a blue dye as per Formula VIIa

### APPLICATION EXAMPLE 6 (olive shade)

0.2 % of a red dye of formula (I)
0.4 % of a yellow dye as per Example 4
0.3 % of a blue dye as per Formula VIb.

### APPLICATION EXAMPLE 7 (red shade)

0.2 % of a red dye of formula (I)
0.4 % of a yellow dye as per Example 4

### APPLICATION EXAMPLE 8 (reddish orange shade)

0.3 % of a red dye of formula (I)
0.9 % of a orange dye as per Example 6

### APPLICATION EXAMPLE 9 (orange shade)

0.1 % of a red dye of formula (I)
0.5 % of a yellow dye as per Example 6

### APPLICATION EXAMPLE 10 (red orange shade)

0.5 % of a red dye of formula (I)
0.9 % of a yellow dye as per Example 4

### APPLICATION EXAMPLE 11 (light orange shade)

0.2 % of a red dye of formula (I)
0.4 % of a yellow dye as per Example 4

### APPLICATION EXAMPLE 12 (violet blue shade)

0.2 % of a red dye of formula (I)
0.6 % of a blue dye as per Formula V a

### APPLICATION EXAMPLE 13 (violet blue shade)

0.3 % of a red dye of formula (I)
0.6 % of a blue dye as per Formula V a

### APPLICATION EXAMPLE 14 (reddish blue shade)

0.1 % of a red dye of formula (I)
0.6 % of a blue dye as per Formula V a

### APPLICATION EXAMPLE 15 (violet shade)

0.5 % of a red dye of formula (I)
0.3 % of a blue dye as per Formula VIIa

### APPLICATION EXAMPLE 16 (violet shade)

0.2 % of a red dye of formula (I)
0.3 % of a blue dye as per Formula VIa.

## Claims

1. Trichromatic or bichromatic dyeing process for dyeing or printing hydroxy-group-containing or nitrogen-containing organic substrates **characterized by** using a dye mixture comprising at least one red-dyeing compound of the formula (I) and at least one yellow-dyeing compound or orange-dyeing compound or one blue-dyeing compound.

2. Trichromatic dyeing process according to Claim 1, **characterized in that** it comprises using a dye mixture comprising at least one yellow (or orange)-dyeing compound of the formula (II) wherein
R₄ and R₅ signify independently from each other H or -SO₃H,
A signifies a group of formula (i) or (ia)
wherein
X is a halogen radical and
Y signifies -CH=CH₂ or -CH₂CH₂-Z, wherein Z is a radical which can be eliminated by alkali,
R₆ and R₇ signify independently from each other H; unsubstituted C₁₋₄alkyl or substituted C₁₋₄alkyl,
B signifies
wherein R₈ signifies C₁₋₄alkyl; -NH₂ or -NHC₁₋₄alkyl,
and the asterisk marks the bond to the -N=N- group;
and/or at least one yellow-dyeing compounds or orange-dyeing compounds of formula (IV) wherein
R₁₃ signifies H; methyl; methoxy, ethoxy; -NHCONH₂ or -NHCOCH₃,
R₁₄ signifies H; methyl; methoxy or ethoxy,
RG signifies
wherein
R₁₅ signifies H or chlorine,
Y signifies -CH=CH₂ or -CH₂CH₂-Z, wherein Z is a radical which can be eliminated by alkali, and may be bonded in a meta- or in para-position with respect to the azo group.

3. Trichromatic dyeing process according to Claim 1, **characterized in that** it comprises using a dye mixture comprising at least one blue-dyeing compound of formula (VI) in which
R₂₁ is H or -COOH,
each of R₂₂ and R₂₄ is independently H; -COOH; -SO₃H; -NHCOCH₃; -NHCOCHY₂-CH₂Y₁: -NHCOCY₂=CH₂ or -NHCOCH₂Y₁.
R₂₃ -COOH,
Y, ₁ is chlorine; bromine; -OSO₃H or -SSO₃H and
Y₂ is H; chlorine or bromine;
and/or at least one blue-dyeing compound of formula (VI) in which
Y signifies -CH=CH₂ or -CH₂CH₂-Z, wherein Z is a radical which can be eliminated by alkali,
R₂₅ signifies H or -SO₃H,
R₂₆ signifies H or -SO₃H;
and/or at least one blue-dyeing compound of formula (VII) wherein
each Y signifies independently from each other -CH=CH₂ or -CH₂CH₂-Z, wherein Z is a radical which can be eliminated by alkali,
R₂₇ and R₂₈ are independently from each other H; unsubstituted C₁₋₄alkyl or substituted C₁₋₄alkyl.

4. Trichromatic dyeing process according to Claim 1-3, **characterized by** using a dye mixture comprising at least one yellow (or orange)-dyeing compound of formula (IIa), (IIb) and/or (IIc) wherein A is or and/or at least one yellow-dyeing compounds or orange-dyeing compounds of formula (IVa) or (IVb) wherein RG is

5. Trichromatic dyeing process according to Claim 1-4, **characterized by** using a dye mixture comprising at least one blue-dyeing compound of formula (Va) or (Vb) and/or at least one blue-dyeing compounds of formula (VIa) or (VIb) and/or at least one blue-dyeing compound of formula (VIIa)

6. A dye mixture comprising at least one red-dyeing compound of the formula (1) and at least one yellow-dyeing compound or orange-dyeing compound or one blue-dyeing compound wherein the at least one yellow (or orange)-dyeing compound is of the formula (II) wherein
R₄ and R₅ signify independently from each other H or -SO₃H,
A signifies a group of formula (i) or (ia)
wherein
X is a halogen radical and
Y signifies -CH=CH₂ or -CH₂CH₂-Z, wherein Z is a radical which can be eliminated by alkali,
R₆ and R₇ signify independently from each other H; unsubstituted C₁₋₄alkyl or substituted C₁₋₄alkyl,
B signifies
wherein R₈ signifies C₁₋₄alkyl; -NH₂ or -NHC₁₋₄alkyl,
and the asterisk marks the bond to the -N=N- group;
and/or at the least one yellow-dyeing compounds or orange-dyeing compounds is of formula (IV) wherein
R₁₃ signifies H; methyl; methoxy, ethoxy; -NHCONH₂ or -NHCOCH₃,
R₁₄ signifies H; methyl; methoxy or ethoxy,
RG signifies
wherein
R₁₅ signifies H or chlorine,
Y signifies -CH=CH₂ or -CH₂CH₂-Z, wherein Z is a radical which can be eliminated by alkali, and may be bonded in a meta- or in para-position with respect to the azo group.
and the at least one blue-dyeing compound is of formula (VI) in which
R₂₁ is H or -COOH,
each of R₂₂ and R₂₄ is independently H; -COOH; -SO₃H: -NHCOCH₃; -NHCOCHY₂-CH₂Y₁; -NHCOCY₂=CH₂ or -NHCOCH₂Y₁.
R₂₃ -COOH,
Y₁, is chlorine; bromine; -OSO₃H or -SSO₃H and
Y₂ is H; chlorine or bromine;
and/or the at least one blue-dyeing compound is of formula (VI) in which
Y signifies -CH=CH₂ or -CH₂CH₂-Z, wherein Z is a radical which can be eliminated by alkali,
R₂₅ signifies H or -SO₃H,
R₂₆ signifies H or -SO₃H;
and/or the at least one blue-dyeing compound is of formula (VII) wherein
each Y signifies independently from each other -CH=CH₂ or -CH₂CH₂-Z, wherein Z is a radical which can be eliminated by alkali,
R₂₇ and R₂₈ are independently from each other H; unsubstituted C₁₋₄alkyl or substituted C₁₋₄alkyl.

7. A dye mixture according to Claim 6, **characterized in that** the at least one yellow (or orange)-dyeing compound is of formula (IIa), (IIb) and/or (IIc) wherein A is or and/or at least one yellow-dyeing compounds or orange-dyeing compounds of formula (IVa) or (IVb) wherein RG is

8. A dye mixture according to Claim 6, **characterized in that** the at least one blue-dyeing compound is of formula (Va) or (Vb) and/or at least one blue-dyeing compounds of formula (VIa) or (VIb) and/or at least one blue-dyeing compound of formula (VIIa)

9. Substrates consisting of hydroxy-group-containing or nitrogen-containing organic substrates dyed or printed by a trichromatic dyeing process as claimed in any of Claims 1-5.

10. Substrates consisting of hydroxy-group-containing or nitrogen-containing organic substrates dyed or printed with a dye mixture according to any of Claims 6-8.

## Patentansprüche

1. Trichromie- oder Bichromiefärbeverfahren zum Färben oder Bedrucken von hydroxygruppenhaltigen oder stickstoffhaltigen organischen Substraten, **gekennzeichnet durch** Verwendung einer Farbstoffmischung, enthaltend mindestens eine rotfärbende Verbindung der Formel (I) und mindestens eine gelbfärbende Verbindung oder orangefärbende Verbindung oder eine blaufärbende Verbindung.

2. Trichromiefärbeverfahren nach Anspruch 1, **dadurch gekennzeichnet, dass** man eine Farbstoffmischung verwendet, die mindestens eine gelb- (oder orange)färbende Verbindung der Formel (II) worin die Formelglieder jeweils folgende Bedeutung haben:
R₄ und R₅ bezeichnen jeweils unabhängig voneinander H oder -SO₃H,
A bezeichnet eine Gruppe der Formel (i) oder (ia)
worin die Formelglieder jeweils folgende Bedeutung haben:
X ist ein Halogenrest und
Y bezeichnet -CH=CH₂ oder -CH₂CH₂-Z, wobei Z ein alkalisch eliminierbarer Rest ist,
R₆ und R₇ bezeichnen unabhängig voneinander H oder gegebenenfalls substituiertes C₁₋₄-Alkyl,
B bezeichnet
worin R₈ C₁₋₄-Alkyl, -NH₂ oder -NHC₁₋₄-Alkyl bezeichnet,
und das Sternchen die Verknüpfung zur -N=N-Gruppe markiert;
und/oder mindestens eine gelbfärbende Verbindung oder orangefärbende Verbindung der Formel (IV) worin die Formelglieder jeweils folgende Bedeutung haben:
R₁₃ bezeichnet H, Methyl, Methoxy, Ethoxy, -NHCONH₂ oder -NHCOCH₃,
R₁₄ bezeichnet H, Methyl, Methoxy oder Ethoxy,
RG bezeichnet
worin die Formelglieder jeweils folgende Bedeutung haben:
R₁₅ bezeichnet H oder Chlor,
Y bezeichnet -CH=CH₂ oder -CH₂CH₂-Z, wobei Z ein alkalisch eliminierbarer Rest ist, und in meta- oder para-Stellung zur Azogruppe stehen kann, enthält.

3. Trichromiefärbeverfahren nach Anspruch 1, **dadurch gekennzeichnet, dass** man eine Farbstoffmischung verwendet, die mindestens eine blaufärbende Verbindung der Formel (VI) worin die Formelglieder jeweils folgende Bedeutung haben:
R₂₁ ist H oder -COOH,
R₂₂ und R₂₄ sind jeweils unabhängig voneinander H, -COOH, -SO₃H, -NHCOCH₃, -NHCOCHY₂-CH₂Y₁, -NHCOCY₂=CH₂ oder -NHCOCH₂Y₁,
R₂₃ -COOH,
Y₁ ist Chlor, Brom, -OSO₃H oder -SSO₃H und
Y₂ ist H, Chlor oder Brom,
und/oder mindestens eine blaufärbende Verbindung der Formel (VI) worin die Formelglieder jeweils folgende Bedeutung haben:
Y bezeichnet -CH=CH₂ oder -CH₂CH₂-Z, wobei Z ein alkalisch eliminierbarer Rest ist,
R₂₅ bezeichnet H oder -SO₃H,
R₂₆ bezeichnet H oder -SO₃H,
und/oder mindestens eine blaufärbende Verbindung der Formel (VII) worin die Formelglieder jeweils folgende Bedeutung haben:
jedes Y bezeichnet unabhängig voneinander -CH=CH₂ oder -CH₂CH₂-Z, wobei Z ein alkalisch eliminierbarer Rest ist,
R₂₇ und R₂₈ sind jeweils unabhängig voneinander H oder gegebenenfalls substituiertes C₁₋₄-Alkyl,
enthält.

4. Trichromiefärbeverfahren nach Anspruch 1-3, **gekennzeichnet durch** Verwendung einer Farbstoffmischung, enthaltend mindestens eine gelb- (oder orange)färbende Verbindung der Formel (IIa), (IIb) und/oder (IIc) wobei A für oder steht
und/oder mindestens eine gelbfärbende Verbindung oder orangefärbende Verbindung der Formel (IVa) oder (IVb) wobei RG für steht.

5. Trichromiefärbeverfahren nach Anspruch 1-4, **gekennzeichnet durch** Verwendung einer Farbstoffmischung, enthaltend mindestens eine blaufärbende Verbindung der Formel (Va) oder (Vb) und/oder mindestens eine blaufärbende Verbindung der Formel (VIa) oder (VIb) und/oder mindestens eine blaufärbende Verbindung der Formel (VIIa)

6. Farbstoffmischung, enthaltend mindestens eine rotfärbende Verbindung der Formel (I) und mindestens eine gelbfärbende Verbindung oder orangefärbende Verbindung oder eine blaufärbende Verbindung, wobei die mindestens eine gelb- (oder orange)färbende Verbindung der Formel (II) entspricht worin die Formelglieder jeweils folgende Bedeutung haben:
R₄ und R₅ bezeichnen jeweils unabhängig voneinander H oder -SO₃H,
A bezeichnet eine Gruppe der Formel (i) oder (ia)
worin die Formelglieder jeweils folgende Bedeutung haben:
X ist ein Halogenrest und
Y bezeichnet -CH=CH₂ oder -CH₂CH₂-Z, wobei Z ein alkalisch eliminierbarer Rest ist,
R₆ und R₇ bezeichnen unabhängig voneinander H oder gegebenenfalls substituiertes C₁₋₄-Alkyl,
B bezeichnet
worin R₈ C₁₋₄-Alkyl, -NH₂ oder -NHC₁₋₄-Alkyl bezeichnet,
und das Sternchen die Verknüpfung zur -N=N-Gruppe markiert;
und/oder die mindestens eine gelbfärbende Verbindung oder orangefärbende Verbindung der Formel (IV) entspricht worin die Formelglieder jeweils folgende Bedeutung haben:
R₁₃ bezeichnet H, Methyl, Methoxy, Ethoxy, -NHCONH₂ oder -NHCOCH₃,
R₁₄ bezeichnet H, Methyl, Methoxy oder Ethoxy,
RG bezeichnet
worin die Formelglieder jeweils folgende Bedeutung haben:
R₁₅ bezeichnet H oder Chlor,
Y bezeichnet -CH=CH₂ oder -CH₂CH₂-Z, wobei Z ein alkalisch eliminierbarer Rest ist, und in meta- oder para-Stellung zur Azogruppe stehen kann,
und die mindestens eine blaufärbende Verbindung der Formel (VI) entspricht worin die Formelglieder jeweils folgende Bedeutung haben:
R₂₁ ist H oder -COOH,
R₂₂ und R₂₄ sind jeweils unabhängig voneinander H, -COOH, -SO₃H, -NHCOCH₃, -NHCOCHY₂-CH₂Y₁" -NHCOCY₂=CH₂ oder -NHCOCH₂Y₁,
R₂₃ -COOH,
Y₁ ist Chlor, Brom, -OSO₃H oder -SSO₃H und
Y₂ ist H, Chlor oder Brom,
und/oder die mindestens eine blaufärbende Verbindung der Formel (VI) entspricht worin die Formelglieder jeweils folgende Bedeutung haben:
Y bezeichnet -CH=CH₂ oder -CH₂CH₂-Z, wobei Z ein alkalisch eliminierbarer Rest ist,
R₂₅ bezeichnet H oder -SO₃H,
R₂₆ bezeichnet H oder -SO₃H,
und/oder die mindestens eine blaufärbende Verbindung der Formel (VII) entspricht worin die Formelglieder jeweils folgende Bedeutung haben:
jedes Y bezeichnet unabhängig voneinander -CH=CH₂ oder -CH₂CH₂-Z, wobei Z ein alkalisch eliminierbarer Rest ist,
R₂₇ und R₂₈ sind jeweils unabhängig voneinander H oder gegebenenfalls substituiertes C₁₋₄-Alkyl.

7. Farbstoffmischung nach Anspruch 6, **dadurch gekennzeichnet, dass** die mindestens eine gelb-(oder orange)färbende Verbindung der Formel (IIa), (IIb) und/oder (IIc) entspricht wobei A für oder steht
und/oder mindestens eine gelbfärbende Verbindung oder orangefärbende Verbindung der Formel (IVa) oder (IVb) wobei RG für steht.

8. Farbstoffmischung nach Anspruch 6, **dadurch gekennzeichnet, dass** die mindestens eine blaufärbende Verbindung der Formel (Va) oder (Vb) entspricht und/oder mindestens eine blaufärbende Verbindung der Formel (VIa) oder (VIb) und/oder mindestens eine blaufärbende Verbindung der Formel (VIIa)

9. Substrate aus hydroxygruppenhaltigen oder stickstoffhaltigen organischen Substraten, gefärbt oder bedruckt nach einem Trichromiefärbeverfahren gemäß einem der Ansprüche 1-5.

10. Substrate aus hydroxygruppenhaltigen oder stickstoffhaltigen organischen Substraten, gefärbt oder bedruckt mit einer Farbstoffmischung gemäß einem der Ansprüche 6-8.

## Revendications

1. Procédé de coloration trichromatique ou bichromatique pour colorer ou imprimer des substrats organiques contenant un groupe hydroxy ou contenant un azote **caractérisé par** l'utilisation d'un mélange de colorants comprenant au moins un composé colorant rouge de formule (I) et au moins un composé colorant jaune ou composé colorant orange ou un composé colorant bleu.

2. Procédé de coloration trichromatique selon la revendication 1, **caractérisé en ce qu'**il comprend l'utilisation d'un mélange de colorants comprenant au moins un composé colorant jaune (ou orange) de formule (II) dans laquelle
R₄ et R₅ désignent indépendamment l' un de l'autre H ou -SO₃H,
A désigne un groupe de formule (i) ou (ia) où
X est un radical halogène et
Y désigne -CH=CH₂ ou -CH₂CH₂-Z, où Z est un radical qui peut être éliminé par un alcali,
R₆ et R₇ désignent indépendamment l'un de l'autre H ; un alkyle en C₁₋₄ non substitué ou un alkyle en C₁₋₄ substitué,
B désigne où R₈ désigne un alkyle en C₁₋₄ ; -NH₂ ou -NH (alkyle en C₁₋₄) ,
et l'astérisque indique la liaison au groupe -N=N- ; et/ou au moins un composé colorant jaune ou composé colorant orange de formule (IV) dans laquelle
R₁₃ désigne H ; un méthyle ; un méthoxy, un éthoxy ; -NHCONH₂ ou -NHCOCH₃,
R₁₄ désigne H ; un méthyle ; un méthoxy ou un éthoxy, RG désigne où
R₁₅ désigne H ou un chlore,
Y désigne -CH=CH₂ ou -CH₂CH₂-Z, où Z est un radical qui peut être éliminé par un alcali, et peut être lié en position méta ou para par rapport au groupe azo.

3. Procédé de coloration trichromatique selon la revendication 1, **caractérisé en ce qu'**il comprend l'utilisation d'un mélange de colorants comprenant au moins un composé colorant bleu de formule (VI) dans laquelle
R₂₁ est H ou -COOH,
chacun de R₂₂ et R₂₄ est indépendamment H ; -COOH ; -SO₃H ; -NHCOCH₃ ; -NHCOCHY₂-CH₂Y₁ ; -NHCOCY₂=CH₂ ou -NHCOCH₂Y₁,
R₂₃ -COOH,
Y₁, est un chlore ; un brome ; -OSO₃H ou -SSO₃H et
Y₂ est H ; un chlore ou un brome ;
et/ou au moins un composé colorant bleu de formule (VI) dans laquelle
Y désigne -CH=CH₂ ou -CH₂CH₂-Z, où Z est un radical qui peut être éliminé par un alcali,
R₂₅ désigne H ou -SO₃H,
R₂₆ désigne H ou -SO₃H ;
et/ou au moins un composé colorant bleu de formule (VII) dans laquelle
chaque Y désigne indépendamment des autres -CH=CH₂ ou -CH₂CH₂-Z, où Z est un radical qui peut être éliminé par un alcali,
R₂₇ et R₂₈ sont indépendamment l'un de l'autre H ; un alkyle en C₁₋₄ non substitué ou un alkyle en C₁₋₄ substitué.

4. Procédé de coloration trichromatique selon la revendication 1 à 3, **caractérisé par** l'utilisation d'un mélange de colorants comprenant au moins un composé colorant jaune (ou orange) de formule (IIa), (IIb) et/ou (IIc) où A est ou et/ou au moins un composé colorant jaune ou composé colorant orange de formule (IVa) ou (IVb) où RG est

5. Procédé de coloration trichromatique selon la revendication 1 à 4, **caractérisé par** l'utilisation d'un mélange de colorants comprenant au moins un composé colorant bleu de formule (Va) ou (Vb) et/ou au moins un composé colorant bleu de formule (VIa) ou (VIb) et/ou au moins un composé colorant bleu de formule (VIIa)

6. Mélange de colorants comprenant au moins un composé colorant rouge de formule (I) et au moins un composé colorant jaune ou composé colorant orange ou un composé colorant bleu où l'au moins un composé colorant jaune (ou orange) est de formule (II) dans laquelle
R₄ et R₅ désignent indépendamment l'un de l'autre H ou -SO₃H,
A désigne un groupe de formule (i) ou (ia)
où
X est un radical halogène et
Y désigne -CH=CH₂ ou -CH₂CH₂-Z, où Z est un radical qui peut être éliminé par un alcali,
R₆ et R₇ désignent indépendamment l'un de l'autre H ; un alkyle en C₁₋₄ non substitué ou un alkyle en C₁₋₄ substitué,
B désigne où R₈ désigne un alkyle en C₁₋₄ ; -NH₂ ou -NH (alkyle en C₁₋₄) ,
et l'astérisque indique la liaison au groupe -N=N- ; et/ou au moins un composé colorant jaune ou composé colorant orange est de formule (IV)
dans laquelle
R₁₃ désigne H ; un méthyle ; un méthoxy, un éthoxy ; -NHCONH₂ ou -NHCOCH₃,
R₁₄ désigne H ; un méthyle ; un méthoxy ou un éthoxy, RG désigne
où
R₁₅ désigne H ou un chlore,
Y désigne -CH=CH₂ ou -CH₂CH₂-Z, où Z est un radical qui peut être éliminé par un alcali, et peut être lié en position méta ou para par rapport au groupe azo,
et l'au moins un composé colorant bleu est de formule (VI) dans laquelle
R₂₁ est H ou -COOH,
chacun de R₂₂ et R₂₄ est indépendamment H ; -COOH ; -SO₃H ; -NHCOCH₃ ; -NHCOCHY₂-CH₂Y₁ ; -NHCOCY₂=CH₂ ou -NHCOCH₂Y₁,
R₂₃ -COOH,
Y₁ est un chlore ; un brome ; -OSO₃H ou -SSO₃H et
Y₂ est H ; un chlore ou un brome ;
et/ou l'au moins un composé colorant bleu est de formule (VI) dans laquelle
Y désigne -CH=CH₂ ou -CH₂CH₂-Z, où Z est un radical qui peut être éliminé par un alcali,
R₂₅ désigne H ou -SO₃H,
R₂₆ désigne H ou -SO₃H ;
et/ou l'au moins un composé colorant bleu est de formule (VII) dans laquelle
chaque Y désigne indépendamment des autres -CH=CH₂ ou -CH₂CH₂-Z, où Z est un radical qui peut être éliminé par un alcali,
R₂₇ et R₂₈ sont indépendamment l'un de l'autre H ; un alkyle en C₁₋₄ non substitué ou un alkyle en C₁₋₄ substitué.

7. Mélange de colorants selon la revendication 6, **caractérisé en ce que** l'au moins un composé colorant jaune (ou orange) est de formule (IIa), (IIb) et/ou (IIc) où A est ou
et/ou au moins un composé colorant jaune ou composé colorant orange de formule (IVa) ou (IVb) où RG est

8. Mélange de colorants selon la revendication 6, **caractérisé en ce que** l'au moins un composé colorant bleu est de formule (Va) ou (Vb) et/ou au moins un composé colorant bleu de formule (VIa) ou (VIb) et/ou au moins un composé colorant bleu de formule (VIIa)

9. Substrats constitués de substrats organiques contenant un groupe hydroxy ou contenant un azote colorés ou imprimés par un procédé de coloration trichromatique selon l'une quelconque des revendications 1 à 5.

10. Substrats constitués de substrats organiques contenant un groupe hydroxy ou contenant un azote colorés ou imprimés avec un mélange de colorants selon l'une quelconque des revendications 6 à 8.
